



US007045263B2

(12) **United States Patent**  
**Zhu et al.**

(10) **Patent No.:** **US 7,045,263 B2**  
(45) **Date of Patent:** **May 16, 2006**

(54) **PHOTORECEPTOR FOR  
ELECTROPHOTOGRAPHY HAVING A SALT  
OF AN ELECTRON TRANSPORT  
COMPOUND**

(75) Inventors: **Jiayi Zhu**, Woodbury, MN (US);  
**Nusrallah Jubran**, St. Paul, MN (US);  
**Kam Wah Law**, Woodbury, MN (US);  
**Zbigniew Tokarski**, Woodbury, MN  
(US)

(73) Assignee: **Samsung Electronics Co. Ltd.**, Suwon  
(KR)

(\*) Notice: Subject to any disclaimer, the term of this  
patent is extended or adjusted under 35  
U.S.C. 154(b) by 172 days.

(21) Appl. No.: **10/664,203**

(22) Filed: **Sep. 17, 2003**

(65) **Prior Publication Data**

US 2004/0101773 A1 May 27, 2004

**Related U.S. Application Data**

(60) Provisional application No. 60/429,716, filed on Nov.  
27, 2002.

(51) **Int. Cl.**  
**G03G 5/047** (2006.01)

(52) **U.S. Cl.** ..... **430/58.45**; 430/58.05;  
430/59.4; 430/64; 430/66; 430/126; 399/159

(58) **Field of Classification Search** ..... 430/58.45,  
430/58.05, 59.4, 64, 66, 126; 399/159  
See application file for complete search history.

(56) **References Cited**

U.S. PATENT DOCUMENTS

3,909,260 A 9/1975 Seoka et al.  
4,015,984 A 4/1977 Ohta et al.

|                 |         |                                 |
|-----------------|---------|---------------------------------|
| 4,152,152 A     | 5/1979  | Contois et al.                  |
| 4,264,696 A     | 4/1981  | Kawashima et al.                |
| 4,845,263 A *   | 7/1989  | Ong et al. ..... 558/427        |
| 4,933,246 A     | 6/1990  | Teuscher                        |
| 5,045,421 A     | 9/1991  | Fuse et al.                     |
| 5,204,201 A     | 4/1993  | Schank et al.                   |
| 5,288,573 A     | 2/1994  | Hung et al.                     |
| 5,342,718 A     | 8/1994  | Nousho et al.                   |
| 5,389,477 A *   | 2/1995  | Tsuchiya et al. ..... 430/58.15 |
| 5,693,442 A     | 12/1997 | Weiss et al.                    |
| 5,731,117 A     | 3/1998  | Ferrar et al.                   |
| 6,045,957 A     | 4/2000  | Takeshima et al.                |
| 6,066,425 A     | 5/2000  | Ferrar et al.                   |
| 6,187,491 B1    | 2/2001  | Ferrar et al.                   |
| 6,383,699 B1    | 5/2002  | Yuh et al.                      |
| 2003/0087172 A1 | 5/2003  | Zhu et al.                      |

FOREIGN PATENT DOCUMENTS

|    |             |        |
|----|-------------|--------|
| JP | 61-188543   | 8/1986 |
| JP | 61188543 A  | 8/1986 |
| JP | 10-239874   | 9/1998 |
| JP | 2000-242023 | 9/2000 |
| JP | 2000-267321 | 9/2000 |

\* cited by examiner

Primary Examiner—Mark A. Chapman

(74) Attorney, Agent, or Firm—Patterson, Thuente, Skaar & Christensen, P.A.

(57) **ABSTRACT**

This invention relates to an improved organophotoreceptor that comprises an electrically conductive substrate; a photoconductive element comprising a charge generation compound and a salt of an electron transport compound. In some embodiments, the photoconductive element has a photoconductive layer with the charge generation compound and an overcoat layer with the salt of the electron transport compound in which the photoconductive layer is on the electrically conductive substrate and the overcoat layer is on the photoconductive layer.

**27 Claims, No Drawings**

## 1

**PHOTORECEPTOR FOR  
ELECTROPHOTOGRAPHY HAVING A SALT  
OF AN ELECTRON TRANSPORT  
COMPOUND**

**CROSS REFERENCE TO RELATED  
APPLICATIONS**

This application claims priority to copending Provisional U.S. Patent Application Ser. No. 60/429,716 to Zhu et al. filed on Nov. 27, 2002, entitled "Novel Overcoat Layer Having A Salt Of An Electron Transport Compound," incorporated herein by reference.

**FIELD OF THE INVENTION**

This invention relates to organophotoreceptors suitable for use in electrophotography and, more specifically, to organophotoreceptors comprising a salt of an electron transport compound.

**BACKGROUND OF THE INVENTION**

In electrophotography, an organophotoreceptor in the form of a plate, disk, sheet, belt, drum or the like having an electrically insulating photoconductive element on an electrically conductive substrate is imaged by first uniformly electrostatically charging the surface of the photoconductive layer, and then exposing the charged surface to a pattern of light. The light exposure selectively dissipates the charge in the illuminated areas where light strikes the surface, thereby forming a pattern of charged and uncharged areas, referred to as a latent image. A liquid or solid toner is then provided in the vicinity of the latent image, and toner droplets or particles deposit in the vicinity of either the charged or uncharged areas to create a toned image on the surface of the photoconductive layer. The resulting toned image can be transferred to a suitable ultimate or intermediate receiving surface, such as paper, or the photoconductive layer can operate as an ultimate receptor for the image. The imaging process can be repeated many times to complete a single image, for example, by overlaying images of distinct color components or effect shadow images, such as overlaying images of distinct colors to form a full color final image, and/or to reproduce additional images.

Both single layer and multilayer photoconductive elements have been used. In single layer embodiments, a charge transport material and charge generating material are combined with a polymeric binder and then deposited on the electrically conductive substrate. In multilayer embodiments, the charge transport material and charge generating material are present in the element in separate layers, each of which can optionally be combined with a polymeric binder, deposited on the electrically conductive substrate. Two arrangements are possible. In one two-layer arrangement (the "dual layer" arrangement), the charge generating layer is deposited on the electrically conductive substrate and the charge transport layer is deposited on top of the charge generating layer. In an alternate two-layer arrangement (the "inverted dual layer" arrangement), the order of the charge transport layer and charge generating layer is reversed.

In both the single and multilayer photoconductive elements, the purpose of the charge generating material is to generate charge carriers (i.e., holes and/or electrons) upon exposure to light. The purpose of the charge transport material is to accept at least one type of these charge carriers,

## 2

generally holes, and transport them through the charge transport layer in order to facilitate discharge of a surface charge on the photoconductive element. The charge transport material can be a charge transport compound, an electron transport compound, or a combination of both. When a charge transport compound is used, the charge transport compound accepts the hole carriers and transports them through the layer with the charge transport compound. When an electron transport compound is used, the electron transport compound accepts the electron carriers and transports them through the layer with the electron transport compound.

**SUMMARY OF THE INVENTION**

15 This invention provides a photoconductive element having a salt of an electron transport compound for improving the photoelectrical properties of organophotoreceptors such as " $V_{acc}$ " and " $V_{dis}$ ".

20 In a first aspect, the invention features an organophotoreceptor that comprises:

a) an electrically conductive substrate; and  
b) a photoconductive element comprising a charge generation compound and a salt of an electron transport compound, wherein the photoconductive element is on the electrically conductive substrate. The photoconductive element can comprise a photoconductive layer comprising the charge generation compound and an overcoat layer comprising a salt of an electron transport compound wherein the overcoat layer is on the photoconductive layer.

25 In a second aspect, the invention features an electrophotographic imaging apparatus that comprises (a) a light imaging apparatus; and (b) the above-described organophotoreceptor oriented to receive light from the light imaging component. The apparatus can further comprise a toner dispenser.

30 In a third aspect, the invention features an electrophotographic imaging process that comprises (a) applying an electrical charge to a surface of the above-described organophotoreceptor; (b) imagewise exposing the surface of the organophotoreceptor to radiation to dissipate charge in selected areas and thereby form a pattern of charged and uncharged areas on the surface; (c) contacting the surface with a toner to create a toned image; and (d) transferring the 35 toned image to a substrate.

**DETAILED DESCRIPTION OF PREFERRED  
EMBODIMENTS**

40 Improved organophotoreceptors comprise an electrically photoconductive element comprising at least a charge generating compound and a salt of an electron transport compound. In some embodiments, the photoconductive element comprises an overcoat layer with the salt of the electron

45 transport compound, although alternatively or additionally the salt of the electron transport compound can be in a photoconductive layer. Generally, the overcoat layer is on a photoconductive layer, which can be, for example, a single layer or an inverted dual layer. The overcoat layer can be applied, for example, as a release layer at the surface of the organophotoreceptor. The salt of the electron transport compound in the organophotoreceptor can improve the performance of the organophotoreceptor in electrophotographic applications, especially organophotoreceptors that are 50 designed to operate with a positive surface charge, including applications based on liquid toners. In some embodiments, the overcoat layer with at least one salt of an electron

transport compound provides the desirable properties of high " $V_{acc}$ ", low " $V_{dis}$ ", good mechanical abrasion for cycling, and good chemical resistance to ozone, carrier fluid and contaminants.

The amount of charge that the charge transport composition can accept is indicated by a parameter known as the acceptance voltage or " $V_{acc}$ ", and the retention of that charge upon discharge is indicated by a parameter known as the discharge voltage or " $V_{dis}$ ". To produce high quality images, it is desirable to increase  $V_{acc}$  and to decrease  $V_{dis}$ .

Organophotoreceptors can comprise an overcoat layer that protects the underlying layers from mechanical degradations and attacks by chemicals such as carrier fluid, corona gases, and ozone. Generally, in order for an overcoat layer to provide the desired protection they should possess certain mechanical properties, and generally are applied in a substantially uniform thickness. Additionally, the overcoat material should be selected so as to not adversely affect the photoelectric properties of the organophotoreceptor beyond acceptable amounts.

An overcoat layer generally does not have an uppermost surface having a high conductivity so that a high " $V_{acc}$ " can be obtained and latent image spread (LIS) along the surface is appropriately low. However, the overcoat layers should not possess a high electrical resistivity to electrons from the layers below the overcoat layer, such as a charge generating layer (single layer or inverted dual layer), or to holes from a charge transport layer (dual layer), so that the overcoat layer does not contribute to an undesirably high value for " $V_{dis}$ " or trap charges opposite to the polarity of the photocconductor.

There are overcoat layers for organophotoreceptors described in the art for protecting the underlying layers. Most of them comprise polymeric binders having very low electrical conductivity. As a result, " $V_{dis}$ " of the organophotoreceptors with a polymeric overcoat layer can be adversely affected. In order to improve " $V_{dis}$ " of organophotoreceptors with a polymeric overcoat layer, new methods for increasing conductivity of the polymeric overcoat layers are desirable. There continues to be a need in particular embodiments for additional organophotoreceptors with an overcoat layer that provides a high " $V_{acc}$ ", a low " $V_{dis}$ ", good mechanical abrasion resistance during extended cycling or printing, and good chemical resistance to ozone, carrier fluid and contaminants.

An overcoat layer comprising an electron transport compound for improving photoelectric properties of organophotoreceptors having an overcoat are described further in U.S. patent application Ser. No. 10/396,536, to Zhu, et al., entitled "Organophotoreceptor With An Electron Transport Layer," incorporated herein by reference. Furthermore, it may be desirable to improve electron transport through photoconductive elements, especially for organophotoreceptors used with positive surface charge.

Generally, the electron transport composition has an electron affinity that is large relative to potential electron traps while yielding an appropriate electron mobility in a composite with a polymer. In some embodiments, the electron transport composition has a reduction potential less than  $O_2$ . In general, electron transport compositions are easy to reduce and difficult to oxidize while charge transport compositions generally are easy to oxidize and difficult to reduce. In some embodiments, the electron transport compounds have a room temperature, zero field electron mobility of at least about  $1 \times 10^{-13} \text{ cm}^2/\text{Vs}$ , in further embodiments at least about  $1 \times 10^{-10} \text{ cm}^2/\text{Vs}$ , in additional embodiments at least about  $1 \times 10^{-8} \text{ cm}^2/\text{Vs}$ , and in other embodiments at

least about  $1 \times 10^{-6} \text{ cm}^2/\text{Vs}$ . A person of ordinary skill in the art will recognize that other ranges of electron mobility within the explicit ranges are contemplated and are within the present disclosure.

5 The incorporation of salts of electron transport compounds into the photoconductive element can enhance the performance of the photoconductive element, in particular, with respect to lowering  $V_{dis}$ . The salt of the electron transport compound can be, for example, within a photoconductive layer and/or an overcoat layer. For example, the 10 salt of the electron transport compound generally can comprise a cation and an anion derived from an electron transport compound. Salts refer broadly to compounds that have a dominant degree of ionic bonding at least between two 15 species within the compound, i.e., a cation and an anion. The anion and cation themselves can have covalent bonding within the ions. Also, a salt generally can comprise more than two ions, such as  $MgCl_2$  with three ions.

The organophotoreceptors described herein are particularly 20 useful in laser printers and the like as well as photocopiers, scanners and other electronic devices based on electrophotography. The use of these organophotoreceptors is described in more detail below in the context of laser printer use, although their application in other devices 25 operating by electrophotography can be generalized from the discussion below. To produce high quality images, particularly after multiple cycles, it generally is desirable for the compositions within the respective layers to form a homogeneous solution with a polymeric binder for forming the 30 particular layer and remain approximately homogeneously distributed through the overcoat layer during the cycling of the material.

In electrophotography applications, a charge generating 35 compound within an organophotoreceptor absorbs light to form electron-hole pairs. These electron-hole pairs can be transported over an appropriate time frame under a large electric field to discharge locally a surface charge that is generating the field. The discharge of the field at a particular location results in a surface charge pattern that essentially 40 matches the pattern drawn with the light. This charge pattern then can be used to guide toner deposition. The organophotocconductors described herein are especially effective at transporting charge, and in particular holes from the electron-hole pairs formed by the charge generating compound. 45 Furthermore, a specific electron transport compound can also be used along with the charge transport composition to transport charges. Improved salt forms of electron transport compounds are described herein.

The layer or layers of materials containing the charge 50 generating compound and the appropriate transport compositions are within an organophotoreceptor. To print a two dimensional image using the organophotoreceptor, the organophotoreceptor has a two dimensional surface for forming at least a portion of the image. The imaging process then 55 continues by cycling the organophotoreceptor to complete the formation of the entire image and/or for the processing of subsequent images. The organophotoreceptor may be provided in the form of a plate, a sheet, a flexible belt, a disk, a rigid drum, a sheet around a rigid or compliant drum, or the like.

The organophotoreceptor may include an electrically conductive substrate and a photoconductive element featuring a charge generating layer. The photoconductive element generally 60 comprises a charge generating material that absorbs light to generate electron and hole pairs. The photoconductive element may further comprise a charge transport compound that is effective for transporting holes, i.e., positive

charge carriers. In some embodiments, the photoconductive element has a single layer with both a charge transport composition and a charge generating compound within a polymeric binder. In further embodiments, a charge generating compound is in a charge transport layer distinct from the charge generating layer. Alternatively, the charge generating layer may be intermediate between the charge transport layer and the electrically conductive substrate. A single layer construction with one layer comprising a charge generating compound and a charge transport compound can be particularly suitable for organophotoreceptors used with a positive surface charge.

The organophotoreceptors can be incorporated into an electrophotographic imaging apparatus, such as laser printers. In these devices, an image is formed from physical embodiments and converted to a light image that is scanned onto the organophotoreceptor to form a surface latent image. The surface latent image can be used to attract toner onto the surface of the organophotoreceptor, in which the toner image is the same or the negative of the light image projected onto the organophotoreceptor. The toner can be a liquid toner or a dry toner. The toner is subsequently transferred, from the surface of the organophotoreceptor, to a receiving surface, such as a sheet of paper. After the transfer of the toner, the entire surface is discharged, and the material is ready to cycle again. The imaging apparatus can further comprise, for example, a plurality of support rollers for transporting a paper receiving medium and/or for movement of the photoreceptor, suitable optics to form the light image, a light source, such as a laser, a toner source and delivery system and an appropriate control system.

An electrophotographic imaging process generally can comprise (a) applying an electrical charge to a surface of the above-described organophotoreceptor; (b) imagewise exposing the surface of the organophotoreceptor to radiation to dissipate charge in selected areas and thereby form a pattern of charged and uncharged areas on the surface; (c) exposing the surface with a toner, such as a liquid toner that includes a dispersion of colorant particles in an organic liquid, to attract toner to the charged or discharged regions of the organophotoreceptor to create a toned image; and (d) transferring the toned image to a substrate.

In describing chemicals by structural formulae and group definitions, certain terms are used in a nomenclature format that is chemically acceptable. The terms groups, moiety, and derivatives have specific meanings. The term group indicates that the generically recited chemical material (e.g., alkyl group, stilbenyl group, phenyl group, etc.) may have any substituent thereon which is consistent with the bond structure of that group. For example, alkyl group includes alkyl materials such as methyl ethyl, propyl iso-octyl, dodecyl and the like, and also includes such substituted alkyls such as chloromethyl, dibromoethyl, 1,3-dicyanopropyl, 1,3,5-trihydroxyhexyl, 1,3,5-trifluorocyclohexyl, 1-methoxydodecyl, phenylpropyl and the like. However, as is consistent with such nomenclature, no substitution would be included within the term that would alter the fundamental bond structure of the underlying group. For example, where a stilbenyl group is recited, substitution such as 3-methyl-stilbenyl would be acceptable within the terminology, while substitution of 3,3-dimethylstilbenyl would not be acceptable as that substitution would require the ring bond structure of one of the phenyl group to be altered to a non-aromatic form because of the substitution.

Where the term moiety is used, such as alkyl moiety or phenyl moiety, that terminology indicates that the chemical material is not substituted. For example, the term alkyl

moiety represents only an unsubstituted alkyl hydrocarbon group, whether branched, straight chain, or cyclic. Where the term derivative is used, that terminology indicates that a compound is derived or obtained from another and containing essential elements of the parent substance.

#### Organophotoreceptors

The organophotoreceptor may be, for example, in the form of a plate, a sheet, a flexible belt, a disk, a rigid drum, or a sheet around a rigid or compliant drum, with flexible belts and rigid drums generally being used in commercial embodiments. The organophotoreceptor may comprise, for example, an electrically conductive substrate and on the electrically conductive substrate a photoconductive element in the form of one or more layers. The photoconductive element can further comprise one or more overcoats or undercoats with respect to a photoconductive layer that comprises a charge generating layer and optionally additional layers.

The photoconductive element can comprise both a charge transport compound and a charge generating compound in a polymeric binder, which may or may not be in the same layer, as well as an electron transport compound in some embodiments. For example, the charge transport compound and the charge generating compound can be in a single layer. In other embodiments, however, the photoconductive element comprises a bilayer construction featuring a charge generating layer and a separate charge transport layer. The charge generating layer may be located intermediate between the electrically conductive substrate and the charge transport layer. Alternatively, the photoconductive element may have a structure in which the charge transport layer is intermediate between the electrically conductive substrate and the charge generating layer.

The electrically conductive substrate may be flexible, for example in the form of a flexible web or a belt, or inflexible, for example in the form of a drum. A drum can have a hollow cylindrical structure that provides for attachment of the drum to a drive that rotates the drum during the imaging process. Typically, a flexible electrically conductive substrate comprises an electrically insulating substrate and a thin layer of electrically conductive material onto which the photoconductive material is applied.

The electrically insulating substrate may be paper or a film forming polymer such as polyester (e.g., polyethylene terephthalate or polyethylene naphthalate), polyimide, polysulfone, polypropylene, nylon, polyester, polycarbonate, polyvinyl resin, polyvinyl fluoride, polystyrene and the like. Specific examples of polymers for supporting substrates included, for example, polyethersulfone (Stabar™ S-100, available from ICI), polyvinyl fluoride (Tedlar®, available from E.I. DuPont de Nemours & Company), polybisphenol-A polycarbonate (Makrofol™, available from Mobay Chemical Company) and amorphous polyethylene terephthalate (Melinar™, available from ICI Americas, Inc.). The electrically conductive materials may be graphite, dispersed carbon black, iodide, conductive polymers such as polypyroles and Calgon® conductive polymer 261 (commercially available from Calgon Corporation, Inc., Pittsburgh, Pa.), metals such as aluminum, titanium, chromium, brass, gold, copper, palladium, nickel, or stainless steel, or metal oxide such as tin oxide or indium oxide. In embodiments of particular interest, the electrically conductive material is aluminum. Generally, the photoconductor substrate has a thickness adequate to provide the required mechanical stability. For example, flexible web substrates

generally have a thickness from about 0.01 to about 1 mm, while drum substrates generally have a thickness from about 0.5 mm to about 2 mm.

The charge generating compound is a material which is capable of absorbing light to generate charge carriers, such as a dye or pigment. Non-limiting examples of suitable charge generating compounds include, for example, metal-free phthalocyanines (e.g., ELA 8034 metal-free phthalocyanine available from H.W. Sands, Inc. or Sanyo Color Works, Ltd., CGM-X01), metal phthalocyanines such as titanium phthalocyanine, copper phthalocyanine, oxytitanium phthalocyanine (also referred to as titanyl oxyphthalocyanine, and including any crystalline phase or mixtures of crystalline phases that can act as a charge generating compound), hydroxygallium phthalocyanine, squarylium dyes and pigments, hydroxy-substituted squarylium pigments, perylimides, polynuclear quinones available from Allied Chemical Corporation under the tradename Indofast® Double Scarlet, Indofast® Violet Lake B, Indofast® Brilliant Scarlet and Indofast® Orange, quinacridones available from DuPont under the tradename Monastral™ Red, Monastral™ Violet and Monastral™ Red Y, naphthalene 1,4,5,8-tetracarboxylic acid derived pigments including the perinones, tetrabenzoporphyrins and tetranaphthaloporphyrins, indigo- and thioindigo dyes, benzothioxanthene-derivatives, perylene 3,4,9,10-tetracarboxylic acid derived pigments, polyazo-pigments including bisazo-, trisazo- and tetrakisazo-pigments, polymethine dyes, dyes containing quinazoline groups, tertiary amines, amorphous selenium, selenium alloys such as selenium-tellurium, selenium-tellurium-arsenic and selenium-arsenic, cadmium sulphoselenide, cadmium selenide, cadmium sulphide, and mixtures thereof. For some embodiments, the charge generating compound comprises oxytitanium phthalocyanine (e.g., any phase thereof), hydroxygallium phthalocyanine or a combination thereof.

There are many kinds of charge transport compounds available for electrophotography. For organophotoconductors described herein, any charge transport compound known in the art can be used. Suitable charge transport compounds include, but are not limited to, pyrazoline derivatives, fluorene derivatives, oxadiazole derivatives, stilbene derivatives, hydrazone derivatives, carbazole hydrazone derivatives, triaryl amines, polyvinyl carbazole, polyvinyl pyrene, polyacenaphthylene, or multi-hydrazone compounds comprising at least two hydrazone groups and at least two groups selected from the group consisting of triphenylamine and heterocycles such as carbazole, julolidine, phenothiazine, phenazine, phenoxazine, phenoxathin, thiazole, oxazole, isoxazole, dibenzo(1,4)dioxine, thianthrene, imidazole, benzothiazole, benzotriazole, benzoxazole, benzimidazole, quinoline, isoquinoline, quinoxaline, indole, indazole, pyrrole, purine, pyridine, pyridazine, pyrimidine, pyrazine, triazole, oxadiazole, tetrazole, thiadiazole, benzisoxazole, benzothiazole, dibenzofuran, dibenzothiophene, thiophene, thianaphthene, quinazoline, or cinnoline. In some embodiments, the charge transport compound is a stilbene derivative such as MPCT-10, MPCT-38, and MPCT-46 from Mitsubishi Paper Mills (Tokyo, Japan).

In some embodiments, the photoconductive elements of this invention may contain one or more electron transport compounds. It has been discovered that salts of the electron transport compound can be desirable for use in photoconductive elements, such as in photoconductive layers and/or overcoat layers. The salt of the electron transport compound can be used in the photoconductive element alone or with additional electron transport compounds, such as a neutral

electron transport compound. If a plurality of electron transport compounds is used, the different electron transport compounds can be in the same layer and/or in different layers. In some embodiments, a photoconductive layer comprises a neutral electron transport compound, and an overcoat layer comprises a salt of an electron transport compound.

Generally, for appropriate embodiments, one or more neutral electron transport compounds known in the art can be used. Non-limiting examples of suitable neutral electron transport compound include, for example, bromoaniline, tetracyanoethylene, tetracyanoquinodimethane, 2,4,7-trinitro-9-fluorenone, 2,4,5,7-tetrinitro-9-fluorenone, 2,4,5,7-tetrinitroxanthone, 2,4,8-trinitrothioxanthone, 2,6,8-trinitro-indeno4H-indeno[1,2-b]thiophene-4-one, and 1,3,7-trinitro dibenzothiophene-5,5-dioxide, (2,3-diphenyl-1-indenylidene)malononitrile, 4H-thiopyran-1,1-dioxide and its derivatives such as 4-dicyanomethylene-2,6-diphenyl-4H-thiopyran-1,1-dioxide, 4-dicyanomethylene-2,6-di-m-tolyl-4H-thiopyran-1,1-dioxide, and unsymmetrically substituted 2,6-diaryl-4H-thiopyran-1,1-dioxide such as 4H-1,1-dioxo-2-(p-isopropylphenyl)-6-phenyl-4-(dicyanomethylidene)thiopyran and 4H-1,1-dioxo-2-(p-isopropylphenyl)-6-(2-thienyl)-4-(dicyanomethylidene)thiopyran, derivatives of phospha-2,5-cyclohexadiene, (alkoxycarbonyl-9-fluorenylidene)malononitrile derivatives such as (4-n-butoxycarbonyl-9-fluorenylidene)malononitrile, (4-phenethoxycarbonyl-9-fluorenylidene)malononitrile, (4-carbitoxy-9-fluorenylidene)malononitrile, and diethyl(4-n-butoxycarbonyl-2,7-dinitro-9-fluorenylidene)-malonate, anthraquino dimethane derivatives such as 11,11,12,12-tetracyano-2-alkylanthraquinodimethane and 11,11-dicyano-12,12-bis(ethoxycarbonyl)anthraquinodimethane, anthrone derivatives such as 1-chloro-10-[bis(ethoxycarbonyl)methylene]anthrone, 1,8-dichloro-10-[bis(ethoxycarbonyl)methylene]anthrone, 1,8-dihydroxy-10-[bis(ethoxycarbonyl)methylene]anthrone, and 1-cyano-10-[bis(ethoxycarbonyl)methylene]anthrone, 7-nitro-2-aza-9-fluorenylidene malononitrile, diphenoquinone derivatives, benzoquinone derivatives, naphtoquinone derivatives, quinone derivatives, tetracyanoethylene, 2,4,8-trinitrothioxanthone, dinitrobenzene derivatives, dinitroanthracene derivatives, dinitroacridine derivatives, nitroanthraquinone derivatives, dinitroanthraquinone derivatives, succinic anhydride, maleic anhydride, dibromo maleic anhydride, pyrene derivatives, carbazole derivatives, hydrazone derivatives, N,N-dialkylaniline derivatives, diphenylamine derivatives, triphenylamine derivatives, triphenylmethane derivatives, tetracyanoquinodimethane, 2,4,5,7-tetrinitro-9-fluorenone, 2,4,7-trinitro-9-dicyano methylenefluorenone, 2,4,5,7-tetrinitroxanthone derivatives, and 2,4,8-trinitrothioxanthone derivatives. In some embodiments of interest, the electron transport compound comprises an (alkoxycarbonyl-9-fluorenylidene)malononitrile derivative, such as (4-n-butoxycarbonyl-9-fluorenylidene)malononitrile, (4-phenethoxycarbonyl-9-fluorenylidene)malononitrile, (4-carbitoxy-9-fluorenylidene)malononitrile, and diethyl(4-n-butoxycarbonyl-2,7-dinitro-9-fluorenylidene)-malonate.

It has been discovered that the addition of a salt of an electron transport compound to an overcoat layer having a binder can reduce " $V_{dis}$ " of organophotoreceptors having such an overcoat. Suitable salts of an electron transport compound include, for example, salts comprising a cation and an anion derived from an electron transport compound. Non-limiting examples of suitable cations include  $\text{NH}_4^+$ ,  $\text{K}^+$ ,  $\text{Li}^+$ ,  $\text{Na}^+$ ,  $\text{Rb}^+$ ,  $\text{Cs}^+$ ,  $\text{Ca}^{+2}$ ,  $\text{Mg}^{+2}$ ,  $\text{Sr}^{+2}$ ,  $\text{Ba}^{+2}$ ,  $\text{Al}^{+3}$ ,  $\text{Co}^{+2}$ ,  $\text{Ni}^{+2}$ ,  $\text{Cu}^{+2}$ , and  $\text{Zn}^{+2}$ . Any neutral electron transport com-

pound having an acidic group may be converted by a base into the corresponding anions suitable for this invention. For example, acid anhydride group, carboxylic acid group, sulfonic acid group, and phosphonic acid group in the structure of the electron transport compound known in the art may be converted into a corresponding carboxylate group, carboxylate group, sulfonate group, and phosphonate group respectively. Non-limiting examples of suitable electron transport compounds that can be formed into salts derivatives include, for example, nitro-9-fluorenone derivatives, dinitro-9-fluorenone derivatives, trinitro-9-fluorenone derivatives, tetrinitro-9-fluorenone derivatives, tetracyanoquinodimethane derivatives, 2,4,5,7-tetrinitroxanthone derivatives, 2,4,8-trinitrothioxanthone derivatives, 2,6,8-trinitro-indeno4H-indeno[1,2-b]thiophene-4-one derivatives, and 1,3,7-trinitro-ibenzothiophene-5,5-dioxide, (2,3-diphenyl-1-indenylidene)malononitrile derivatives, 4H-thiopyran-1,1-dioxide derivatives, unsymmetrically substituted 2,6-diaryl-4H-thiopyran-1,1-dioxide, phospha-2,5-cyclohexadiene derivatives, (alkoxycarbonyl-9-fluorenylidene)malononitrile derivatives, anthraquinodimethane derivatives, anthrone derivatives, 7-nitro-2-aza-9-fluorenylidene-malononitrile derivatives, diphenoquinone derivatives, benzoquinone derivatives, naphtoquinone derivatives, quinine derivatives, 2,4,8-trinitrothioxanthone, dinitrobenzene derivatives, dinitroanthracene derivatives, dinitroacridine derivatives, nitroanthraquinone derivatives, succinic anhydride, maleic anhydride, dibromo maleic anhydride, pyrene derivatives, carbazole derivatives, hydrazone derivatives, N,N-dialkylaniline derivatives, diphenylamine derivatives, triphenylamine derivatives, triphenylmethane derivatives, 2,4,7-trinitro-9-dicyanomethylenene fluorenone derivatives, 2,4,5,7-tetrinitroxanthone derivatives, and 2,4,8-trinitrothioxanthone derivatives. In some embodiments of particular interest, the anion of electron transport compound for this invention is selected from the group consisting of the following formula:



To form the salt of the electron transport compound, the acidic electron transport compound can be combined with a

suitable base such that the cation of the base becomes the cation of the salt and the anion of the electron transport compound becomes the anion of the salt. Generally, this formation of the salt is performed in an aqueous solution, for example, by adding an excess of base and adding acid to obtain the salt of the electron transport compound. In some embodiments, the salt can be formed in other solvents, generally polar solvents, such as alcohols. After the salt of the electron transport compound is obtained, if a binder and/or other compound is to be combined with the salt, the binder and/or other compounds can be selected to be soluble and/or dispersable in an appropriate solution along with the salt.

In general, an electron transport compound and a UV light stabilizer can have a synergistic relationship for providing desired electron flow within the photoconductor. The presence of the UV light stabilizers alters the electron transport properties of the electron transport compounds to improve the electron transporting properties of the composite. UV light stabilizers can be ultraviolet light absorbers or ultraviolet light inhibitors that trap free radicals.

UV light absorbers can absorb ultraviolet radiation and dissipate it as heat. UV light inhibitors are thought to trap free radicals generated by the ultraviolet light and after trapping of the free radicals, subsequently to regenerate active stabilizer moieties with energy dissipation. In view of the synergistic relationship of the UV stabilizers with electron transport compounds, the particular advantages of the UV stabilizers may not be their UV stabilizing abilities, although the UV stabilizing ability may be further advantageous in reducing degradation of the organophotoreceptor over time. While not wanting to be limited by theory, the synergistic relationship contributed by the UV stabilizers may be related to the electronic properties of the compounds, which contribute to the UV stabilizing function, by further contributing to the establishment of electron conduction pathways in combination with the electron transport compounds. In particular, the organophotoreceptors with a combination of the electron transport compound and the UV stabilizer can demonstrate a more stable acceptance voltage  $V_{acc}$  with cycling. The improved synergistic performance of organophotoreceptors with layers comprising both an electron transport compound and a UV stabilizer are described further in copending U.S. patent application Ser. No. 10/425,333 filed on Apr. 28, 2003 to Zhu, entitled "Organophotoreceptor With A Light Stabilizer," incorporated herein by reference.

Non-limiting examples of suitable light stabilizer include, for example, hindered trialkylamines such as Tinuvin 144 and Tinuvin 292 (from Ciba Specialty Chemicals, Terrytown, N.Y.), hindered alkoxydialkylamines such as Tinuvin 123 (from Ciba Specialty Chemicals), benzotriazoles such as Tinuvan 328, Tinuvin 900 and Tinuvin 928 (from Ciba Specialty Chemicals), benzophenones such as Sanduvor 3041 (from Clariant Corp., Charlotte, N.C.), nickel compounds such as Arbestab (from Robinson Brothers Ltd, West Midlands, Great Britain), salicylates, cyanocinnamates, benzylidene malonates, benzoates, oxanilides such as Sanduvor VSU (from Clariant Corp., Charlotte, N.C.), triazines such as Cyagard UV-1164 (from Cytec Industries Inc., N.J.), polymeric sterically hindered amines such as Luchem (from Atochem North America, Buffalo, N.Y.). In some embodiments, the light stabilizer is selected from the group consisting of hindered trialkylamines having the following formula:



where R<sub>1</sub>, R<sub>2</sub>, R<sub>3</sub>, R<sub>4</sub>, R<sub>5</sub>, R<sub>6</sub>, R<sub>7</sub>, R<sub>8</sub>, R<sub>9</sub>, R<sub>10</sub>, R<sub>11</sub>, R<sub>12</sub>, R<sub>13</sub>, R<sub>14</sub>, R<sub>15</sub> are, independently, hydrogen, alkyl group, or ester, or ether group; and R<sub>5</sub>, R<sub>9</sub>, and R<sub>14</sub> are, independently, alkyl group; and X is a linking group selected from the group consisting of  $-\text{O}-\text{CO}-\text{(CH}_2\text{)}_m-\text{CO}-\text{O}-$  where m is between 2 to 20.

The binder generally is capable of dispersing or dissolving the charge transport compound (in the case of the charge transport layer or a single layer photoconductive element construction), the charge generating compound (in the case of the charge generating layer or a single layer photoconductive element construction) and/or an electron transport compound for appropriate embodiments. Examples of suitable binders for both the charge generating layer and charge transport layer generally include, for example, polystyrene-co-butadiene, polystyrene-co-acrylonitrile, modified acrylic polymers, polyvinyl acetate, styrene-alkyd resins, soya-alkyl resins, polyvinylchloride, polyvinylidene chloride, polyacrylonitrile, polycarbonates, polyacrylic acid, polyacrylates, polymethacrylates, styrene polymers, polyvinyl butyral, alkyd resins, polyamides, polyurethanes, polyesters, polysulfones, polyethers, polyketones, phenoxy resins, epoxy resins, silicone resins, polysiloxanes, poly(hydroxy-ether) resins, polyhydroxystyrene resins, novolak, poly(phenylglycidyl ether)-co-dicyclopentadiene, copolymers of monomers used in the above-mentioned polymers, and combinations thereof. In some embodiments, polycarbonate binders and/or polyvinyl butyral binders are of particular interest. Examples of suitable polycarbonate binders include, for example, polycarbonate A which is derived from bisphenol-A, polycarbonate Z, which is derived from cyclohexylidene bisphenol, polycarbonate C, which is derived from methylbisphenol A, and polyestercarbonates. Suitable polyvinyl butyral binders include, for example, BX-1 and BX-5 from Sekisui Chemical Co. Ltd., Japan. The above binders may be solvent-based or water-based. In some embodiments, overcoat binders are water-based or water-borne polymeric binder. Non-limiting examples of water-based polymeric binders suitable for the overcoats described herein are polyurethanes such as Andura<sup>TM</sup>-50, -100, and -200 from Air Products, Shakopee, Minn. 55379, urethane-acrylic resin such as Hybridur<sup>TM</sup>-560, -570, and -580 from Air Products, epoxy resin such as Ancarez<sup>TM</sup> AR 550 from Air Products, and Beckopox<sup>TM</sup> from Solutia Inc., St. Louis, Mo.

Suitable optional additives for any one or more of the layers include, for example, antioxidants, coupling agents, dispersing agents, curing agents, surfactants and combinations thereof.

The photoconductive element overall typically has a thickness from about 10 to about 45 microns and in some embodiments from about 12 microns to about 40 microns. In the dual layer embodiments having a separate charge generating layer and a separate charge transport layer, charge generation layer generally has a thickness from about 0.5 to about 2 microns, and the charge transport layer generally has a thickness from about 5 to about 35 microns. In embodiments in which the charge transport compound and the charge generating compound are in the same layer, the layer with the charge generating compound and the charge transport composition generally has a thickness from about 7 to about 30 microns. In embodiments with a distinct electron transport layer, the electron transport layer has an average thickness from about 0.5 microns to about 10 microns and in further embodiments from about 1 micron to about 3 microns. In general, an electron transport overcoat layer can increase mechanical abrasion resistance, increases resistance to carrier liquid and atmospheric moisture, and decreases degradation of the photoreceptor by corona gases. A person of ordinary skill in the art will recognize that additional ranges of thickness within the explicit ranges above are contemplated and are within the present disclosure.

Generally, for the organophotoreceptors described herein, the charge generation compound is in an amount from about 0.5 to about 25 weight percent, in further embodiments in an amount from about 1 to about 15 weight percent and in other embodiments in an amount from about 2 to about 10 weight percent, based on the weight of the photoconductive layer. The charge transport compound is in an amount from about 10 to about 80 weight percent, based on the weight of the photoconductive layer, in further embodiments in an amount from about 35 to about 60 weight percent, and in other embodiments from about 45 to about 55 weight percent, based on the weight of the photoconductive layer. The optional electron transport compound, when present, can be in an amount of at least about 2 weight percent, in other embodiments from about 2.5 to about 25 weight percent, based on the weight of the photoconductive layer, and in further embodiments in an amount from about 4 to about 20 weight percent, based on the weight of the photoconductive layer. The binder is in an amount from about 15 to about 80 weight percent, based on the weight of the photoconductive layer, and in further embodiments in an amount from about 20 to about 75 weight percent, based on the weight of the photoconductive layer. A person of ordinary skill in the art will recognize that additional ranges within the explicit ranges of compositions are contemplated and are within the present disclosure.

For the dual layer embodiments with a separate charge generating layer and a charge transport layer, the charge generation layer generally comprises a binder in an amount from about 10 to about 90 weight percent, in further embodiments from about 15 to about 80 weight percent and in some embodiments in an amount from about 20 to about 75 weight percent, based on the weight of the charge generation layer. The optional electron transport compound in the charge generating layer, if present, generally can be in an amount of at least about 2.5 weight percent, in further embodiments from about 4 to about 30 weight percent and in other embodiments in an amount from about 10 to about 25 weight percent, based on the weight of the charge generating layer. The charge transport layer generally comprises a binder in an amount from about 20 weight percent to about 70 weight percent and in further embodiments in an amount from about 30 weight percent to about 50 weight percent. A person of

ordinary skill in the art will recognize that additional ranges of binder concentrations for the dual layer embodiments within the explicit ranges above are contemplated and are within the present disclosure.

For the embodiments with a single layer having a charge generating compound and a charge transport compound, the photoconductive layer generally comprises a binder, a charge transport compound and a charge generation compound. The charge generation compound can be in an amount from about 0.05 to about 25 weight percent and in further embodiment in an amount from about 2 to about 15 weight percent, based on the weight of the photoconductive layer. The charge transport compound can be in an amount from about 10 to about 80 weight percent, in other embodiments from about 25 to about 65 weight percent, in additional embodiments from about 30 to about 60 weight percent and in further embodiments in an amount of from about 35 to about 55 weight percent, based on the weight of the photoconductive layer, with the remainder of the photoconductive layer comprising the binder, and optionally additives, such as any conventional additives. A single layer with a charge transport composition and a charge generating compound generally comprises a binder in an amount from about 10 weight percent to about 75 weight percent, in other embodiments from about 20 weight percent to about 60 weight percent, and in further embodiments from about 25 weight percent to about 50 weight percent. Optionally, the layer with the charge generating compound and the charge transport compound may comprise an electron transport compound. The optional electron transport compound, if present, generally can be in an amount of at least about 2.5 weight percent, in further embodiments from about 4 to about 30 weight percent, in additional embodiments from about 5 to about 25 weight percent and in other embodiments in an amount from about 10 to about 20 weight percent, based on the weight of the photoconductive layer. A person of ordinary skill in the art will recognize that additional composition ranges within the explicit compositions ranges for the layers above are contemplated and are within the present disclosure.

In general, any layer with an electron transport layer can advantageously further include a UV light stabilizer. In particular, the electron transport layer generally can comprise an electron transport compound, a binder and an optional UV light stabilizer. An overcoat layer comprising an electron transport compound is described further in copending U.S. patent application Ser. No. 10/396,536 to Zhu et al. entitled, "Organophotoreceptor With An Electron Transport Layer," incorporated herein by reference. For example, an electron transport compound as described above may be used in the release layer of the photoconductors described herein. The electron transport compound in an electron transport layer can be in an amount from about 1 to about 50 weight percent, in some embodiments from about 5 to about 40 weight percent, in further embodiments, from about 10 to about 30 weight percent, and in other embodiments in an amount from about 20 to about 25 weight percent, based on the weight of the electron transport layer. A person of ordinary skill in the art will recognize that additional ranges of compositions within the explicit ranges are contemplated and are within the present disclosure.

The UV light stabilizer, if present, in any of one or more appropriate layers of the photoconductor generally is in an amount from about 0.5 to about 25 weight percent and in some embodiments in an amount from about 1 to about 10 weight percent, based on the weight of the particular layer.

A person of ordinary skill in the art will recognize that additional ranges of compositions within the explicit ranges are contemplated and are within the present disclosure.

For example, the photoconductive layer may be formed by dispersing or dissolving the components, such as one or more of a charge generating compound, a charge transport compound, an electron transport compound, a UV light stabilizer, and a polymeric binder in organic solvent, coating the dispersion and/or solution on the respective underlying layer and drying the coating. In particular, the components can be dispersed by high shear homogenization, ball-milling, attritor milling, high energy bead (sand) milling or other size reduction processes or mixing means known in the art for effecting particle size reduction in forming a dispersion. For photoconductive elements with multiple layers, generally the layers can be applied sequentially to form the desired structure.

The photoreceptor may optionally have one or more additional layers as well. An additional layer can be, for example, a sub-layer or an overcoat layer, such as a barrier layer, a release layer, a protective layer, or an adhesive layer. A release layer or a protective layer may form the uppermost layer of the photoconductor element. A barrier layer may be sandwiched between the release layer and the photoconductive element or used to overcoat the photoconductive element. The barrier layer provides protection from abrasion to the underlayers. An adhesive layer locates and improves the adhesion between a photoconductive element, a barrier layer and a release layer, or any combination thereof. A sub-layer is a charge blocking layer and locates between the electrically conductive substrate and the photoconductive element. The sub-layer may also improve the adhesion between the electrically conductive substrate and the photoconductive element.

The binder for the overcoat layer may be, for example, polymers such as fluorinated polymer, siloxane polymer, fluorosilicone polymer, silane, polyethylene, polypropylene, polyacrylate, poly(methyl methacrylate-co-methacrylic acid), urethane resin, urethane-epoxy resin, acrylated-urethane resins, urethane-acrylic resin, epoxy resins, or a combination thereof. The above binders may be solvent-based or water-based. In some embodiments, overcoat binders are water-based or waterborne polymeric binder. Non-limiting examples of water-based polymeric binders suitable for the overcoats described herein are polyurethanes such as Andurat<sup>TM</sup>-50, -100, and -200 from Air Products, Shakopee, Minn. 55379, urethane-acrylic resin such as Hybridur<sup>TM</sup>-560, -570, and -580 from Air Products, epoxy resin such as Ancarez<sup>TM</sup> AR 550 from Air Products, and Beckopox<sup>TM</sup> from Solutia Inc., St. Louis, Mo. The overcoat binders of particular interest comprise water-based polyurethane. However, most of the above polymer binders have low electrical conductivity and thus provide high  $V_{dis}$ , when unmodified.

Suitable barrier layers include, for example, coatings such as crosslinkable siloxanol-colloidal silica coating and hydroxylated silsesquioxane-colloidal silica coating, and organic binders such as polyvinyl alcohol, methyl vinyl ether/maleic anhydride copolymer, casein, polyvinyl pyrrolidone, polyacrylic acid, gelatin, starch, polyurethanes, polyimides, polyesters, polyamides, polyvinyl acetate, polyvinyl chloride, polyvinylidene chloride, polycarbonates, polyvinyl butyral, polyvinyl acetoacetate, polyvinyl formal, polyacrylonitrile, polymethyl methacrylate, polyacrylates, polyvinyl carbazoles, copolymers of monomers used in the above-mentioned polymers, vinyl chloride/vinyl acetate/vinyl alcohol terpolymers, vinyl chloride/vinyl acetate/maleic acid terpolymers, ethylene/vinyl acetate copolymers,

15

vinyl chloride/vinylidene chloride copolymers, cellulose polymers, and mixtures thereof. The above barrier layer polymers optionally may contain small inorganic particles such as fumed silica, silica, titania, alumina, zirconia, or a combination thereof. Barrier layers are described further in U.S. Pat. No. 6,001,522 to Woo et al., entitled "Barrier Layer For Photoconductor Elements Comprising An Organic Polymer And Silica," incorporated herein by reference. The release layer topcoat may comprise any release layer composition known in the art. In some embodiments, the release layer is a fluorinated polymer, siloxane polymer, fluorosilicone polymer, silane, polyethylene, polypropylene, polyacrylate, or a combination thereof. The release layers can comprise crosslinked polymers.

The release layer may comprise, for example, any release layer composition known in the art. In some embodiments, the release layer comprises a fluorinated polymer, siloxane polymer, fluorosilicone polymer, polysilane, polyethylene, polypropylene, polyacrylate, poly(methyl methacrylate-co-methacrylic acid), urethane resins, urethane-epoxy resins, acrylated-urethane resins, urethane-acrylic resins, or a combination thereof. In further embodiments, the release layers comprise crosslinked polymers.

The protective layer can protect the organophotoreceptor from chemical and mechanical degradation. The protective layer may comprise any protective layer composition known in the art. In some embodiments, the protective layer is a fluorinated polymer, siloxane polymer, fluorosilicone polymer, polysilane, polyethylene, polypropylene, polyacrylate, poly(methyl methacrylate-co-methacrylic acid), urethane resins, urethane-epoxy resins, acrylated-urethane resins, urethane-acrylic resins, or a combination thereof. In some embodiments of particular interest, the protective layers are crosslinked polymers.

An overcoat layer may comprise an electron transport compound as described further in copending U.S. patent application Ser. No. 10/396,536, filed on Mar. 25, 2003 to Zhu et al. entitled, "Organoreceptor With An Electron Transport Layer," incorporated herein by reference. As described herein, salts of electron transport compounds can be effectively substituted into overcoat layers to improve the photoconductive properties of the organophotoreceptor with the overcoat. For example, an electron transport compound, as described above, may be used in the release layer of this invention. The electron transport compound in the overcoat layer can be in an amount from about 1 to about 50 weight percent, in some embodiments in an amount from about 2 to about 40 weight percent, in additional embodiments from about 5 to about 30 weight percent, and in other embodiments in an amount from about 10 to about 20 weight percent, based on the weight of the release layer. A person of ordinary skill in the art will recognize that additional ranges of composition within the explicit ranges are contemplated and are within the present disclosure.

Generally, adhesive layers comprise a film forming polymer, such as polyester, polyvinylbutyral, polyvinylpyrrolidone, polyurethane, polymethyl methacrylate, poly(hydroxy amino ether) and the like.

Sub-layers can comprise, for example, polyvinylbutyral, organosilanes, hydrolyzable silanes, epoxy resins, polyesters, polyamides, polyurethanes, silicones and the like. In some embodiments, the sub-layer has a dry thickness between about 20 Angstroms and about 2,000 Angstroms. Sublayers containing metal oxide conductive particles can be between about 1 and about 25 microns thick. A person of ordinary skill in the art will recognize that additional ranges

16

of compositions and thickness within the explicit ranges are contemplated and are within the present disclosure.

The organophotoreceptors as described herein are suitable for use in an imaging process with either dry or liquid toner development. For example, any dry toners and liquid toners known in the art may be used in the process and the apparatus of this invention. Liquid toner development can be desirable because it offers the advantages of providing higher resolution images and requiring lower energy for image fixing compared to dry toners. Examples of suitable liquid toners are known in the art. Liquid toners generally comprise toner particles dispersed in a carrier liquid. The toner particles can comprise a colorant/pigment, a resin binder, and/or a charge director. In some embodiments of liquid toner, a resin to pigment ratio can be from 1:1 to 10:1, and in other embodiments, from 4:1 to 8:1. Liquid toners are described further in Published U.S. patent application Ser. No. 2002/0,128,349, entitled "Liquid Inks Comprising A Stable Organosol," Ser. No. 2002/0,086,916, entitled "Liquid Inks Comprising Treated Colorant Particles," and Ser. No. 2002/0,197,552, entitled "Phase Change Developer For Liquid Electrophotography," all three of which are incorporated herein by reference.

The invention will now be described further by way of the following examples.

## EXAMPLES

### Example 1

#### Synthesis of Electron Transport Compounds

This example describes the synthesis or procurement of electron transport compounds including in some embodiments salts of electron transport compounds for the formation of organophotoreceptors.

#### Preparation of (4-n-Butoxycarbonyl-9-fluorenylidene)Malononitrile

A 460 g quantity of concentrated sulfuric acid (4.7 moles, analytical grade, commercially obtained from Sigma-Aldrich, Milwaukee, Wis.) and 100 g of diphenic acid (0.41 mole, commercially obtained from Acros Fisher Scientific Company Inc., Hanover Park, Ill.) were added to a 1-liter 3-neck round bottom flask, equipped with a thermometer, mechanical stirrer and a reflux condenser. Using a heating mantle, the flask was heated to 135–145° C. for 12 minutes, and then cooled to room temperature. After cooling to room temperature, the solution was added to a 4-liter Erlenmeyer flask containing 3 liter of water. The mixture was stirred mechanically and was boiled gently for one hour. A yellow solid was filtered out hot, washed with hot water until the pH of the wash-water was neutral, and was air-dried overnight. The yellow solid was fluorenone-4-carboxylic acid. The yield was 75 g (80%). The product was then characterized. The melting point (m.p.) was found to be 223–224° C. A <sup>1</sup>H-NMR spectrum of fluorenone-4-carboxylic acid was obtained in d<sub>6</sub>-DMSO solvent with a 300 MHz NMR from Bruker Instrument. The peaks were found at (ppm) δ=7.39–7.50 (m, 2H); δ=7.79–7.70 (q, 2H); δ=7.74–7.85 (d, 1H); δ=7.88–8.00 (d, 1H); and δ=8.18–8.30 (d, 1H), where doublet, t is triplet, m is multiplet, dd is doublet, q is quintet.

A 70 g (0.312 mole) quantity of fluorenone-4-carboxylic acid, 480 g (6.5 mole) of n-butanol (commercially obtained from Fisher Scientific Company Inc., Hanover Park, Ill.), 1000 ml of toluene and 4 ml of concentrated sulfuric acid

were added to a 2-liter round bottom flask equipped with a mechanical stirrer and a reflux condenser with a Dean Stark apparatus. The solution was refluxed for 5 hours with aggressive agitation and refluxing, during which time about 6 g of water were collected in the Dean Stark apparatus. The flask was cooled to room temperature. The solvents were evaporated, and the residue was added, with agitation, to 4-liter of a 3% sodium bicarbonate aqueous solution. The solid was filtered off, washed with water until the pH of the wash-water was neutral, and dried in a hood overnight. The product was n-butyl fluorenone-4-carboxylate ester. The yield was 70 g (80%). A <sup>1</sup>H-NMR spectrum of n-butyl fluorenone-4-carboxylate ester was obtained in CDCl<sub>3</sub> with a 300 MHz NMR from Bruker Instrument. The peaks were found at (ppm) δ=0.87–1.09 (t, 3H); δ=1.42–1.70 (m, 2H); δ=1.75–1.88 (q, 2H); δ=4.26–4.64 (t, 2H); δ=7.29–7.45 (m, 2H); δ=7.46–7.58 (m, 1H); δ=7.60–7.68 (dd, 1H); δ=7.75–7.82 (dd, 1H); δ=7.90–8.00 (dd, 1H); δ=8.25–8.35 (dd, 1H).

A 70 g (0.25 mole) quantity of n-butyl fluorenone-4-carboxylate ester, 750 ml of absolute methanol, 37 g (0.55 mole) of malononitrile (commercially obtained from Sigma-Aldrich, Milwaukee, Wis.), 20 drops of piperidine (commercially obtained from Sigma-Aldrich, Milwaukee, Wis.) were added to a 2-liter, 3-neck round bottom flask equipped with a mechanical stirrer and a reflux condenser. The solution was refluxed for 8 hours. Then, the flask was cooled to room temperature. The orange crude product was filtered, washed twice with 70 ml of methanol and once with 150 ml of water, and dried overnight in a hood. The orange crude product was recrystallized from a mixture of 600 ml of acetone and 300 ml of methanol using activated charcoal. The flask was placed at 0° C. for 16 hours. The crystals were filtered and dried in a vacuum oven at 50° C. for 6 hours to obtain 60 g of pure (4-n-butoxycarbonyl-9-fluorenylidene) malononitrile. The melting point (m.p.) of the solid was found to be 99–100° C. A <sup>1</sup>H-NMR spectrum of (4-n-butoxycarbonyl-9-fluorenylidene)malononitrile was obtained in CDCl<sub>3</sub> with a 300 MHz NMR from Bruker Instruments. The peaks were found at (ppm) δ=0.74–1.16 (t, 3H); δ=1.38–1.72 (m, 2H); δ=1.70–1.90 (q, 2H); δ=4.29–4.55 (t, 2H); δ=7.31–7.43 (m, 2H); δ=7.45–7.58 (m, 1H); δ=7.81–7.91 (dd, 1H); δ=8.15–8.25 (dd, 1H); δ=8.42–8.52 (dd, 1H); δ=8.56–8.66 (dd, 1H).

#### Preparation of 9-Fluorenone-4-Carboxylic Acid

A 460 g quantity of concentrated sulfuric acid (4.7 moles, analytical grade, commercially obtained from Sigma-Aldrich, Milwaukee, Wis.) and 100 g of diphenic acid (0.41 mole, commercially obtained from Acros Fisher Scientific Company Inc., Hanover Park, Ill.) were added to a 1-liter 3-neck round bottom flask, equipped with a thermometer, a mechanical stirrer and a reflux condenser. Using a heating mantle, the flask was heated to 135–145° C. for 12 minutes, and then cooled to room temperature. After cooled to room temperature, the solution was added to a 4-liter Erlenmeyer flask containing 3 liters of water. The mixture was stirred mechanically and was boiled gently for one hour. A yellow solid was filtered out hot, washed with hot water until the pH of the washing water was neutral, and dried in the air overnight. The yellow solid was fluorenone-4-carboxylic acid. A 75 g quantity of product was obtained for a yield of 80%. The product was found to have a melting point of 223–224° C. A <sup>1</sup>H-NMR spectrum of fluorenone-4-carboxylic acid in d<sub>6</sub>-DMSO was obtained with a 300 MHz NMR from Bruker Instruments. The peaks were found at (in ppm) δ=7.39–7.50 (m, 2H); δ=7.79–7.70 (q, 2H); δ=7.74–7.85 (d,

1H); δ=7.88–8.00 (d, 1H); and δ=8.18–8.30 (d, 1H), where d is doublet, t is triplet, m is multiplet; dd is double doublet, q is quintet. This precursor was used to synthesize electron transport compounds, as described in the following.

5 Preparation of (4-Carboxy-9-Fluorenylidene)malononitrile A 208 g quantity of 9-fluorenone-4-carboxylic acid (0.93 mole), 3 liters of methanol (obtained from Acros Fisher Scientific Company Inc., Hanover Park, Ill.), 237.8 g of malononitrile (3.6 mole, purchased from Aldrich Chemicals Co.) and 2.81 g of piperidine (0.033 mole, obtained from Aldrich Chemicals Co.) were added to a 5-liter 3-neck round bottom flask equipped with a reflux condenser and a mechanical stirrer. The solution was refluxed overnight. Then, the flask was cooled to room temperature, and an orange product was filtered off. The orange product was stirred in 1 liter of methanol, boiled for half an hour, filtered hot, washed with 100 ml of methanol, and then dried in a vacuum oven for 8 hours at 60° C. This compound can be used to form salts with an anion of Formula (1) above.

#### Preparation of Sodium Salt of (4-Carboxy-9-Fluorenylidene)malononitrile

A 5 g quantity of (4-carboxy-9-fluorenylidene)malononitrile and 95 g of distilled water were added to an 8 oz jar. 25 Then, solid sodium hydroxide was added in excess until all solid went into solution. A solution of 1N HCl was added until the pH dropped from 10–11 to 7–8. Then, the solution was filtered, and the filtrate was used for further evaluation and incorporation into photoreceptors.

#### Preparation of Ammonium Salt of (4-Carboxy-9-Fluorenylidene)malononitrile

A 1 g quantity of (4-carboxy-9-fluorenylidene)malononitrile and 99 g of distilled water were added to an 8 oz jar. 35 Then, an excess of ammonium hydroxide solution was added until all solid went into solution. A solution of 1N HCl was added until the pH dropped from 10–11 to 7–8. Then, the solution was filtered, and the filtrate was used for further evaluation and incorporation into photoreceptors.

#### Preparation of 2,7-Dinitrofluorenone-4-Carboxylic Acid

2,7-Dinitrofluorenone-4-carboxylic acid is prepared by the following method. 9-Fluorenone-4-carboxylic acid (11.2 g, 0.05 moles) is placed in a 500 ml round bottom flask. Then, 300 ml of red fuming nitric acid is added to the flask at room temperature over a period of 10 minutes. This can then be followed by the addition of 50 ml of concentrated sulfuric acid over a 5 minutes period. The resulting solution is stirred at room temperature for 10 minutes and then poured slowly into 1.5 liter of ice cold water with constant stirring. The solid product is collected by filtration, washed with 5% aqueous hydrochloric acid solution, and then dried in a vacuum at 60° C. for 24 hours.

#### Preparation of (2,7-Dinitrofluorenone-4-Carboxylic Acid) malononitrile

A 1 mole quantity of 2,7-dinitrofluorenone-4-carboxylic acid, 3 liters of methanol, 3.6 mole of malononitrile (purchased from Aldrich Chemicals Co.) and 2.81 g of piperidine (0.033 mole, obtained from Aldrich Chemicals Co.) is 60 added to a 5-liter 3-neck round bottom flask equipped with a reflux condenser and a mechanical stirrer. The solution is refluxed overnight. Then, the flask is cooled to room temperature, and an orange product is filtered off. The orange product is stirred in 1 liter of methanol, boiled for half an hour, filtered hot, washed with 100 ml of methanol, and then dried in a vacuum oven for 8 hours at 60° C. The product (2,7-dinitrofluorenone-4-carboxylic acid)malononitrile is 65

19

obtained. The product compound can be used to form salts with an anion of Formula (2) above.

Preparation of Sodium Salt of (2,7-Dinitrofluorenone-4-Carboxylic Acid)malononitrile

Sodium salt of (2,7-dinitrofluorenone-4-carboxylic acid) malononitrile may be prepared by the following method. A 5 g quantity of (2,7-dinitrofluorenone-4-carboxylic acid) malononitrile and 95 g of distilled water is added to an 8 oz jar. Solid sodium hydroxide is added in excess until all solid goes into solution. A solution of 1N HCl is added until the pH drops from 10-11 to 7-8. Then the solution is filtered, and the filtrate can be used for further evaluation and incorporation into photoreceptors.

Preparation of Ammonium Salt of (2,7-Dinitrofluorenone-4-Carboxylic Acid)Malononitrile

A 1 g quantity of (2,7-dinitrofluorenone-4-carboxylic acid) malononitrile and 99 g of distilled water is added to an 8 oz jar. Ammonium hydroxide solution is added in excess until all solid goes into solution. A solution of 1N HCl is added until the pH drops from 10-11 to 7-8. Then, the solution is filtered, and the filtrate can be used for further evaluation and incorporation into photoreceptors.

2,4-Dinitrobenzenesulfonic acid, sodium salt

2,4-Dinitrobenzenesulfonic acid, sodium salt (catalog # 25,993-4) may be obtained commercially from Aldrich, Milwaukee, Wis. This compound can be used to form salts with the structure of Formula (3) above.

Example 2

Preparation of Organophotoreceptors

This example describes the preparation of five organophotoreceptor samples and three comparative samples. These samples and comparative samples are evaluated in the following Examples.

Comparative Sample A

Comparative Sample A was a single layer organophotoreceptor having a 76.2 micron (3 mil) thick polyester substrate with a layer of vapor-coated aluminum (commercially obtained from CP Films, Martinsville, Va.). The coating solution for the single layer organophotoreceptor was prepared by pre-mixing 892.5 g of 20 weight % (4-n-butoxy-carbonyl-9-fluorenylidene)malononitrile dissolved in tetrahydrofuran (commercially obtained from Aldrich, Milwaukee, Wis.), 2475.2 g of 25 weight % MPCT-10 (a charge transfer compound, commercially obtained from Mitsubishi Paper Mills, Tokyo, Japan) dissolved in tetrahydrofuran, 2128.9 g of 14 weight % polyvinyl butyral resins (BX-1, commercially obtained from Sekisui Chemical Co. Ltd., Japan) dissolved in tetrahydrofuran, 158.67 g of 15 weight % Tinuvin®-292 and 130.9 g of 15 weight % Tinuvin®-928 (both commercially available from Ciba Specialty Chemicals, Inc., Terrytown, N.Y.) dissolved in tetrahydrofuran, and 939.9 g of tetrahydrofuran. A 273.9 g quantity of a CGM mill-base containing 19 weight % of titanyl oxyphthalocyanine (commercially obtained from H.W. Sands Corp., Jupiter, Fla.) and a polyvinyl butyral resin (BX-5, commercially obtained from Sekisui Chemical Co. Ltd., Japan) at a weight ratio of 2.3:1 was then added to the above coating solution. The CGM mill-base was obtained by milling 112.7 g of the titanyl oxyphthalocyanine (H.W. Sands Corp., Jupiter, Fla.) with 49 g of the polyvinyl butyral resin (BX-5) in 651 g of methylethylketone on a horizontal sand mill (model LMC12 DCMS, commercially

20

obtained from Netzsch Incorporated, Exton, Pa.) with 1-micron zirconium beads using recycle mode for 6 hours. After mixing of all the coating ingredients, the coating solution was filtered through a 40 micron filter. The filtered coating solution was coated onto the substrate described above by a web coater at a web speed of 10 feet per minute, and the coated web was then dried in a 20 foot oven at a temperature of 110° C. (i.e., 2 minutes of drying at 110° C). The dry coating thickness was measured to be about 13 microns by 10 using a Fischerscope® Multi Measuring System (Version-Permascope by Fischer Technology, Inc., Windsor, Conn.).

Comparative Sample B

Comparative Sample B consisted of an overcoat layer coated on top of an organophotoreceptor as described for Comparative Sample A. The coating solution for the overcoat layer was prepared by premixing 1.0 g of a surfactant BYK®-333 (i.e., a polyether modified poly-dimethyl-siloxane, commercially obtained from BYK®-Chemie USA, Wallingford, Conn.) in 47.4 g of a co-solvent ARCOLSOLV® DPNB (i.e., dipropylene glycol-normal butyl ether, commercially obtained from Lyondell Chemical, Newtown Square, Pa.). In a separate container, 71.4 g of Macekote®-8539 (i.e., a water-dispersed polyurethane, commercially obtained from Mace Adhesives & Coatings Co., Inc., Dudley, Mass.) was diluted with 404.8 g of de-ionized water followed by adding 24.2 g of the premixed solution. After mixing, the coating solution was coated onto an organophotoreceptor substrate as described for Comparative Sample A by using a knife coater with an orifice of 50 micron followed by drying in an oven at 95° C. for 5 minutes.

Comparative Sample C

Comparative Sample C was prepared similarly according to the procedure for Comparative Sample B except that the 35 coating solution had higher percent of solids and the coating was coated directly on a 76.2 micron (3 mil) thick polyester substrate having a layer of vapor-coated aluminum (commercially obtained from CP Films, Martinsville, Va.) such that the final sample did not have a photoconductive layer, 40 which is not needed for resistivity measurements. A premix solution was prepared by premixing 0.5 g of a surfactant BYK®-333 (i.e., a polyether modified poly-dimethyl-siloxane, commercially obtained from BYK®-Chemie USA, Wallingford, Conn.) in 22.5 g of a co-solvent ARCOLSOLV® DPNB (i.e., dipropylene glycol normal butyl ether, commercially obtained from Lyondell Chemical, Newtown Square, Pa.). In a separate container, 7.14 g of Macekote®-8539 (i.e., a water-dispersed polyurethane, commercially obtained from Mace Adhesives & Coatings Co., Inc., Dudley, Mass.) was diluted with 16.7 g of de-ionized water, and the coating solution was formed by adding 1.15 g of the premixed solution to the polyurethane solution. The overcoat was then applied to the substrate as described with comparative sample B. The coating thickness was about 3.1 micron 55 measured by using a Fischerscope® Multi Measuring System (Version-Permascope by Fischer Technology, Inc., Windsor, Conn.).

Sample 1

Sample 1 was prepared similarly according to the procedure for Comparative Sample B except that the coating solution for the overcoat layer was prepared by mixing 28.5 g of the coating solution prepared for Comparative Sample B with 1.5 g of sodium salt of (4-carboxy-9-fluorenylidene) malononitrile.

Sample 2

Sample 2 was prepared similarly according to the procedure for Comparative Sample B except that the coating

solution for the overcoat layer was prepared by mixing 27.0 g of the coating solution prepared for Comparative Sample B with 3.0 g of sodium salt of (4-carboxy-9-fluorenylidene)malononitrile.

### Sample 3

Sample 3 was prepared similarly according to the procedure for Comparative Sample B except that the coating solution for the overcoat layer was prepared by diluting 4.1 g of Macekote®-8539 (i.e., a water-dispersed polyurethane, commercially obtained from Mace Adhesives & Coatings Co., Inc., Dudley, Mass.) with 17.0 g of de-ionized water followed by adding 1.45 g of the premixed solution prepared for Comparative Sample B and 7.5 g of ammonium salt of (4-carboxy-9-fluorenylidene)malononitrile.

### Sample 4

Sample 4 was prepared similarly according to the procedure for Comparative Sample B except that the coating solution for the overcoat layer was prepared by diluting 3.9 g of Macekote®-8539 (i.e., a water-dispersed polyurethane, commercially obtained from Mace Adhesives & Coatings Co., Inc., Dudley, Mass.) with 9.7 g of de-ionized water followed by adding 1.45 g of the premixed solution prepared for Comparative Sample B and 15.0 g of ammonium salt of (4-carboxy-9-fluorenylidene)malononitrile.

### Sample 5

Sample 5 was prepared similarly to Comparative Sample C except that the coating solution for the overcoat layer was prepared by mixing 4.0 g of Macekote®-8539 (i.e., a water-dispersed polyurethane, commercially obtained from Mace Adhesives & Coatings Co., Inc., Dudley, Mass.) with 8.2 g of de-ionized water followed by 0.3 g of the premixed solution of comparative Sample B along with 3.1 g of sodium salt of (4-carboxy-9-fluorenylidene)malononitrile. The dried coating thickness was ~3.1 micron measured by using a Fischerscope® Multi Measuring System (Version-Permascope by Fischer Technology, Inc., Windsor, Conn.).

### Example 3

#### Electrostatic Testing

This example provides results of electrostatic testing on some of the organophotoreceptor samples formed as described in Example 2.

Electrostatic cycling performance of organophotoreceptors described herein with overcoats comprising salt was determined using in-house designed and developed test bed that can test, for example, up to three sample strips wrapped around a 160 mm diameter drum. The results on these samples are indicative of results that would be obtained with other support structures, such as belts, drums and the like, for supporting the organophotoreceptors.

For testing using a 160 mm diameter drum, three coated sample strips, each measuring 50 cm long by 8.8 cm wide, were fastened side-by-side and completely around an aluminum drum (50.3 cm circumference). In some embodiments, at least one of the strips is a control sample that is precision web coated and used as an internal reference point. A control sample with an inverted dual layer structure was used as an internal check of the tester. In this electrostatic cycling tester, the drum rotated at a rate of 8.13 cm/sec (3.2 ips), and the location of each station in the tester (distance and elapsed time per cycle) is given as shown in the following table:

TABLE 1

| Electrostatic test stations around the 160 mm diameter drum at 8.13 cm/sec. |                      |              |                    |                 |
|-----------------------------------------------------------------------------|----------------------|--------------|--------------------|-----------------|
| 5                                                                           | Station              | Degrees      | Total Distance, cm | Total Time, sec |
| 10                                                                          | Front erase bar edge | 0°           | Initial, 0 cm      | Initial, 0 s    |
|                                                                             | Erase Bar            | 0-7.2°       | 0-1.0              | 0-0.12          |
|                                                                             | Scorotron Charger    | 113.1-135.3° | 15.8-18.9          | 1.94-2.33       |
|                                                                             | Laser Strike         | 161.0°       | 22.5               | 2.77            |
|                                                                             | Probe #1             | 181.1°       | 25.3               | 3.11            |
|                                                                             | Probe #2             | 251.2°       | 35.1               | 4.32            |
|                                                                             | Erase bar            | 360°         | 50.3               | 6.19            |

15

The erase bar is an array of laser emitting diodes (LED) with a wavelength of 720 nm that discharges the surface of the organophotoreceptor. The scorotron charger comprises a wire that permits the transfer of a desired amount of charge to the surface of the organophotoreceptor.

From the above table, the first electrostatic probe (Trek 344™ electrostatic meter, Trek, Inc. Medina, N.Y.) is located 0.34 s after the laser strike station and 0.78 s after the scorotron while the second probe (Trek™344 electrostatic meter) is located 1.21 s from the first probe and 1.99 s from the scorotron. All measurements are performed at ambient temperature and relative humidity.

30 Electrostatic measurements were obtained as a compilation of several runs on the test station. The first three diagnostic tests (prodtest initial, VlogE initial, dark decay initial) were designed to evaluate the electrostatic cycling of a new, fresh sample and the last three, identical diagnostic test (prodtest final, VlogE final, dark decay final) are run after cycling of the sample. In addition, measurements were made periodically during the test, as described under "longrun" below. The laser is operated at 780 nm wavelength, 600 dpi, 50 micron spot size, 60 nanoseconds/pixel expose time, 1,800 lines per second scan speed, and a 100% duty cycle. The duty cycle is the percent exposure of the pixel clock period, i.e., the laser is on for the full 60 nanoseconds per pixel at a 100% duty cycle.

#### Electrostatic Test Suite

- 1) PRODTEST: The erase bar was turned on during this diagnostic test and the sample recharged at the beginning of each revolution/cycle (except where indicated as charger off). Charge acceptance ( $V_{acc}$ ) and discharge voltage ( $V_{dis}$ ) were established by subjecting the samples to corona charging (erase bar always on) for three complete drum revolutions (laser off); discharged with the laser @ 780 nm & 600 dpi on the forth revolution (50 um spot size, expose 60 nanoseconds/pixel, run at a scan speed of 1,800 lines per second, and use a 100% duty cycle); completely charged for the next three revolutions (laser off); discharged with only the erase lamp @ 720 nm on the eighth revolution (corona and laser off) to obtain residual voltage ( $V_{res}$ ); and, finally, completely charged for the last three revolutions (laser off). The contrast voltage ( $V_{con}$ ) is the difference between  $V_{acc}$  and  $V_{dis}$  and the functional dark decay ( $V_{dd}$ ) is the difference in charge acceptance potential measured by probes #1 and #2.
- 2) VLOGE: This test measures the photoinduced discharge of the photoconductor to various laser intensity levels by

monitoring the discharge voltage of the sample as a function of the laser power (exposure duration of 50 ns) with fixed exposure times and constant initial potentials. The complete sample was charged and discharged at incremental laser power levels per each drum revolution. A semi-logarithmic plot was generated (voltage versus log E) to identify the sample's functional photosensitivity,  $S_{780mm}$ , and operational power settings.

- 3) DARK DECAY: This test measures the loss of charge acceptance in the dark with time without laser or erase illumination for 90 seconds and can be used as an indicator of i) the injection of residual holes from the charge generation layer to the charge transport layer, ii) the thermal liberation of trapped charges, and iii) the injection of charge from the surface or aluminum ground plane. After the sample has been completely charged, it was stopped and the probes measured the surface voltage over a period of 90 seconds. The decay in the initial voltage was plotted versus time.
- 4) LONGRUN: The sample was electrostatically cycled for 100 drum revolutions according to the following sequence per each sample-drum revolution. The sample was charged by the corona, the laser was cycled on and off (80–100° sections) to discharge a portion of the sample and, finally, the erase lamp discharged the whole sample in preparation for the next cycle. The laser was cycled so that the first section of the sample was never exposed, the second section was always exposed, the third section was never exposed, and the final section was always exposed. This pattern was repeated for a total of 100 drum revolutions, and the data was recorded periodically, after every 5th cycle for the 100 cycle long run.
- 5) After the LONGRUN test, the PRODTEST, VLOGE, DARK DECAY diagnostic tests were run again.

The following Table shows the results from the initial and final prodtest diagnostic tests. The values for the charge acceptance voltage ( $V_{acc}$ , probe #1 average voltage obtained from the third cycle), discharge voltage ( $V_{dis}$ , probe #1 average voltage obtained from the fourth cycle), and the residual voltage ( $V_{res}$ , probe 1, average voltage obtained from the eighth cycle) are reported for the initial and final cycles.

TABLE 1

| Samples  | Electrostatic Results after 100 cycles |           |           |                           |           |           |                  |                  |  |
|----------|----------------------------------------|-----------|-----------|---------------------------|-----------|-----------|------------------|------------------|--|
|          | Prodtest Initial                       |           |           | Prodtest Final-100 Cycles |           |           | Changes          |                  |  |
|          | $V_{acc}$                              | $V_{dis}$ | $V_{res}$ | $V_{acc}$                 | $V_{dis}$ | $V_{res}$ | $\Delta V_{acc}$ | $\Delta V_{dis}$ |  |
| Comp.    | 729                                    | 37        | 14        | 701                       | 37        | 13        | -28              | 0                |  |
| Sample A |                                        |           |           |                           |           |           |                  |                  |  |
| Comp.    | 736                                    | 154       | 143       | 668                       | 233       | 176       | -68              | 79               |  |
| Sample B |                                        |           |           |                           |           |           |                  |                  |  |
| Sample 1 | 745                                    | 135       | 95        | 725                       | 157       | 102       | -20              | 22               |  |
| Sample 2 | 720                                    | 120       | 77        | 665                       | 132       | 78        | -55              | 12               |  |
| Sample 3 | 708                                    | 139       | 95        | 678                       | 171       | 110       | -30              | 32               |  |
| Sample 4 | 715                                    | 124       | 74        | 617                       | 141       | 82        | -98              | 17               |  |

Note:

1)  $V_{acc}$ ,  $V_{dis}$ , and  $V_{res}$  are charge acceptance voltage, discharge voltage, and residual voltage respectively.2)  $\Delta V_{acc}$ ,  $\Delta V_{dis}$  are the differences for charge acceptance, and discharge voltages at the start and the end of the cycling.

3) The electrostatic results for each example listed in the table were average values obtained from 1 to 5 sections of each sample after running electrostatic testing for 1 to 3 times of 100 cycles electrostatic.

## Example 4

## Volume Resistivity Measurement

Volume resistivities of Comparative Sample C and Sample 5 were measured according to ASTM D-257-93 test method, titled "Standard Test Methods for DC Resistance or Conductance of Insulating materials," incorporated herein by reference.

A Resistance/Resistivity Probe (Model-803B by electro-Tech System Inc., Glenside, Pa.) was used to measure the current under an applied voltage of 200 volts. Volume resistivity of the coatings (V.Rm, in ohm.cm) was calculated according the equation provided by the manufacturer as shown below:

$$V.Rm = 7.1 * Rm/t$$

where  $Rm$  was the resistance of the coated material as calculated from the measured current  $I$  (nA) under applied voltage  $U$  (i.e.,  $Rm=U/I$ , where  $U=200$  volt) and  $t$  was the measured thickness (cm) of the coated material.

TABLE 3

| Sample | Time(s)           | Measured Volume Resistance on Overcoat Samples |     |       |       |       |       |       |      |      |      |      |      |      |      |      |      |      |  |
|--------|-------------------|------------------------------------------------|-----|-------|-------|-------|-------|-------|------|------|------|------|------|------|------|------|------|------|--|
|        |                   | 0.5                                            | 1   | 30    | 60    | 90    | 120   | 150   | 180  | 210  | 240  | 270  | 300  | 330  | 360  | 390  | 420  |      |  |
| Comp.  | Current (nA)      | 45                                             | 28  | 4.20  | 2.40  | 1.90  | 1.60  | 1.40  | 1.3  | 1.2  | 1.1  | 1    | 0.9  | 0.9  | 0.8  | 0.8  | 0.8  | 0.8  |  |
| Ex. C  | V. Rm, (ohm · cm) | 1.0                                            | 1.6 | 10.9  | 19.1  | 24.1  | 28.6  | 32.7  | 35.2 | 38.2 | 41.6 | 45.8 | 50.9 | 50.9 | 57.3 | 57.3 | 57.3 | 57.3 |  |
|        | E + 14)           |                                                |     |       |       |       |       |       |      |      |      |      |      |      |      |      |      |      |  |
| Ex. 5  | Current (nA)      | 81                                             | 63  | 24.20 | 21.50 | 20.00 | 19.20 | 18.50 | 18.1 | 17.7 | 17.4 | 17.2 | 16.7 | 16.6 | 16.4 | 16.3 | 16.2 |      |  |
|        | V. Rm (ohm · cm)  | 0.6                                            | 0.8 | 2.0   | 2.2   | 2.4   | 2.5   | 2.6   | 2.6  | 2.7  | 2.7  | 2.8  | 2.8  | 2.9  | 2.9  | 2.9  | 2.9  | 2.9  |  |
|        | E + 14)           |                                                |     |       |       |       |       |       |      |      |      |      |      |      |      |      |      |      |  |

Note:

Data for the measured current were collected immediately after applying the voltage (i.e., at 0.5 and 1 second) and then every 30 seconds up to 7 minutes till the measured current was stabilized.

25

These measurements demonstrate that the sample with the salt of the electron transport compound had significantly lower volume electrical resistivity than the comparative sample without the salt.

As understood by those skilled in the art, additional substitution, variation among substituents, and alternative methods of synthesis and use may be practiced within the scope and intent of the present disclosure of the invention. The embodiments above are intended to be illustrative and not limiting. Additional embodiments are within the claims. Although the present invention has been described with reference to particular embodiments, workers skilled in the art will recognize that changes may be made in form and detail without departing from the spirit and scope of the invention.

What is claimed is:

1. An organophotoreceptor comprising:
  - a) an electrically conductive substrate; and
  - b) a photoconductive element comprising a charge generation compound and a salt of an electron transport compound, wherein the photoconductive element is on the electrically conductive substrate.
2. An organophotoreceptor according to claim 1 wherein the photoconductive element further comprises a charge transport compound.
3. An organophotoreceptor according to claim 1 wherein the charge transport compound comprises a stilbaryl group.
4. An organophotoreceptor according to claim 1 wherein the photoconductive element comprises a photoconductive layer comprising the charge generation compound and an overcoat layer comprising a first binder and the salt of the electron transport compound.
5. An organophotoreceptor according to claim 4 wherein the photoconductive layer further comprises at least an electron transport compound.
6. An organophotoreceptor according to claim 4 wherein the first binder is a water-based polymeric binder.
7. An organophotoreceptor according to claim 4 wherein the amount of the salt in the overcoat layer is between 1% and 50% by weight.
8. An organophotoreceptor according to claim 4 wherein the amount of the salt in the overcoat layer is between 5% and 25% by weight.
9. An organophotoreceptor according to claim 1 wherein the salt comprises an anion of formula



26

-continued



10. An organophotoreceptor according to claim 1 wherein the photoconductive element further comprises a second binder.
11. An organophotoreceptor according to claim 1 further comprising a sublayer located between the electrically conductive substrate and the photoconductive element.
12. An organophotoreceptor according to claim 1 further comprising a barrier layer located between the overcoat layer and the photoconductive element.
13. An electrophotographic imaging apparatus comprising:
  - (a) a light imaging component; and
  - (b) an organophotoreceptor oriented to receive light from the light imaging component, the organophotoreceptor comprising an electrically conductive substrate and a photoconductive element comprising at least a charge generation compound and a salt of an electron transport compound, wherein the photoconductive layer is on the electrically conductive substrate.
14. An electrophotographic imaging apparatus according to claim 13 wherein the photoconductive element further comprises at least an electron transport compound.
15. An electrophotographic imaging apparatus according to claim 13 wherein the photoconductive element comprises an photoconductive layer comprising the charge generation compound, and an overcoat layer comprising a first binder and the salt of the electron transport compound, wherein the overcoat layer is on the photoconductive layer.
16. An electrophotographic imaging apparatus according to claim 15 wherein the first binder is a water-based polymeric binder.
17. An electrophotographic imaging apparatus according to claim 15 wherein the amount of the salt in the overcoat layer is between 1% and 50% by weight.
18. An electrophotographic imaging apparatus according to claim 13 wherein the salt comprises an anion of the following formula:



-continued



19. An electrophotographic imaging apparatus according to claim 13 wherein the photoconductive element further comprises a second binder.

20. An electrophotographic imaging process comprising:

- (a) applying an electrical charge to a surface of an organophotoreceptor comprising an electrically conductive substrate and a photoconductive element comprising a charge generation compound and a salt of an electron transport compound, wherein the photoconductive element is on the electrically conductive substrate;
- (b) imagewise exposing the surface of the organophotoreceptor to radiation to dissipate charge in selected areas and thereby form a pattern of charged and uncharged areas on the surface;
- (c) contacting the surface with a toner to create a toned image; and
- (d) transferring the toned image to a substrate.

21. An electrophotographic imaging process according to claim 20 wherein the photoconductive layer further comprises an electron transport compound.

22. An electrophotographic imaging process according to claim 20 wherein the photoconductive element further comprises a charge transport compound.

23. An electrophotographic imaging process according to claim 20 wherein the photoconductive element comprises a photoconductor layer comprising the charge generation compound and an overcoat layer comprising a first binder and the salt of the electron transport compound, wherein the overcoat layer is on the photoconductive layer.

10

15

20

25

30

35

24. An electrophotographic imaging process according to claim 23 wherein the first binder is a water-based polymeric binder.

25. An electrophotographic imaging process according to claim 24 wherein the amount of the salt in the overcoat layer is between 1% and 50% by weight.

26. An electrophotographic imaging process according to claim 20 wherein the salt comprises an anion of formula



27. An electrophotographic imaging process according to claim 20 wherein the photoconductive element further comprises a second binder.

\* \* \* \* \*